

## UNITED STATES PATENT OFFICE

1,987,467

WATERPROOF ABRASIVE FABRIC AND  
METHOD OF MAKING THE SAMEFrank Joseph Crupi, Brooklyn, N. Y., assignor to  
Behr-Manning Corporation, Brooklyn, N. Y., a  
corporation of New YorkNo Drawing. Application September 15, 1927,  
Serial No. 219,816. Renewed June 11, 1934

15 Claims. (Cl. 51—280)

This invention relates to a method of making an extremely flexible, waterproof, and durable article in the nature of sandpaper or cloth.

At the present time, a large portion of the waterproof sandpaper on the market is used in the automobile industry for body finishing. In the use of sand paper for this purpose the surface to be treated is first well wetted with water and is then sanded with an abrasive fabric which has previously been immersed in water. There are many crevices and other irregular surfaces on an automobile body, and, in order to sand and abrade such parts properly and effectively it is highly desirable that the abrasive fabric should be extremely flexible and should be capable of being crumpled without cracking the abrasive bond. Ordinary waterproof sandpaper when so crumpled frequently caused the abrasive bond to crack due to lack of sufficient flexibility of the fabric, and the sharp edges of such cracks in the crumpled sandpaper cause the formation of relatively deep objectionable scratches on the finished surface of the automobile body.

It is one of the objects of the present invention to prevent the formation of such cracks and to provide a waterproof abrasive fabric which can be crumpled in the wet condition while preserving, throughout, the requisite flexibility.

Heretofore the waterproof abrasive fabric which was generally used had a binder for the abrasive particles consisting of, or at least containing, a gum varnish. When gum varnish was used as the binder, the abrasive fabric or sandpaper was fairly flexible while new. After the passage of a relatively short period of time, however, the fabric began to lose its flexibility due to the oxidation and aging of the varnish binder. When the aforesaid fabrics were used they were therefore relatively brittle and likely to crack fairly easily. Whenever the cracked abrasive bond began to scratch and mar the surface under treatment, indicating that the abrasive fabric was no longer satisfactory or fit for use, a new piece of abrasive fabric had to be substituted. In the effort to prolong the life of such sandpaper, it was proposed to use gums or resins such as kauri, copal, and dammar to increase the adhesion and hardness of the binder. Due, however, to the presence of these relatively brittle gums and resins in the binder, the flexibility of the abrasive fabric was detrimentally reduced. Consequently the abrasive fabrics containing gum-oil varnishes were subject to many disadvantages and were not especially suited for such uses as the finishing of automobile bodies.

I have now discovered a new method of making abrasive fabrics which will overcome the disadvantages noted hereinabove. The new abrasive fabrics will sand the surface under treatment without scratching, will provide a bond between the abrasive particles and the binder, and have practically no tendency to crack, will hold the abrasive particles tenaciously even under wet and crumpled operating conditions, and will preserve an extremely flexible character in such uses.

My invention distinguishes over abrasive fabrics including the gum varnish products in that they will not only have a greater initial flexibility but will also retain the flexibility over a considerable and materially longer period of time.

In the ordinary course of trade it is possible to keep my novel abrasive fabric in regular industrial storage for the usual commercial periods of storing with only negligible effects on the fabric so that the product, after being taken from the storage, still retains substantially all of its original flexibility. Moreover, when the stored fabric is used it is wetted with water and its flexibility is further increased so that it can then be crumpled in use without cracking the abrasive bond.

Generally speaking, my invention consists in covering a surface of a fabric base with a coating or film of polymerized drying oil in which is embedded an abrasive material or a layer of abrasive particles. A film of such oil is superimposed upon a surface of a fabric and constitutes a matrix which adhesively unites or secures a plurality of abrasive particles to the fabric and which completely incorporates and anchors the particles in such a manner that they are held tenaciously to the fabric even under severe rubbing action.

Attention at this point is directed to the fact that the oil used in making my new sandpaper is a polymerized oil as distinguished from non-polymerized oils, i. e. the oil is prepolymerized before it is used. This is a distinction of material importance as the action and behavior of the two types of oil, the polymerized oil on the one hand and the non-polymerized oil on the other, are quite different physically and chemically, especially in their relation to the various elements which make up the finished product.

In the preferred form of my invention the fabric base is first impregnated with a waterproofing agent such as polymerized drying oil or the like. After the impregnated base is properly dried, a coating or film of polymerized drying oil is applied to one of the surfaces of such base. Immediately after the application of the oil abra-

sive particles are sprinkled upon the coated fabric so that a layer of abrasive particles or grains is embedded and incorporated in the film of oil. The abrasive coated fabric is dried and then is 5 preferably covered with a second coat or film of polymerized drying oil so as to completely envelope practically the entire abrasive surface. When this covered surface is dried, the abrasive fabric is ready for use or for sale. In order to 10 obtain the best results in carrying out the aforesaid process, it is preferable to use an oil like linseed or China-wood which is highly refined and purified before polymerization. Such an oil is substantially devoid of free fatty acids and 15 the glycerides of saturated acids.

There are several methods which may be employed for polymerization of the drying oil. The more important of these methods are the usual kettle heating, heating in the absence of oxygen 20 or in an atmosphere of carbonic acid gas, and heating in vacuum. Although any one of these methods may be used, I have found that the best results are obtained by using an oil made by the vacuum method. In the use of the other methods 25 of polymerization the temperature is usually 200 to 300 degrees higher than that employed in the vacuum method. The high heat used in these other methods causes a certain amount of breaking down of molecules with the resultant formation 30 of acids and volatile matter and the production of an impure product. In the vacuum method very little of these acids are formed because of the lower heat employed and because of the removal of the volatile cleavage products by 35 vacuum. With this method there is very little oxidation. The vacuum method, therefore, produces what may theoretically be considered the purest form of polymerization, and the final viscous product is the purest form of drying oil.

40 The polymerization is carried on until the oil has reached its saturation point, i. e., the point just before the oil will begin to gel on further heating. A linseed oil so treated will, generally speaking, have a final iodine number of approximately 122, an acid number of 2 to 3, a saponification value of about 189, and a specific gravity in the neighborhood of 0.974. In using this oil its viscosity is thinned down with a solvent such as petroleum spirits or varnolene until reduced to 45 the desired consistency for coating and for sizing the various fine and coarse grades of abrasive fabrics or sand paper. To hasten the drying of this oil, I have found that the linoleates of cobalt and lead are best suited for this purpose. I may 50 also use the resinate of these metals or a mixture of a paste of linoleates and resinates. The drier that I particularly use is a mixture of a paste of cobalt linoleates containing 5.6% cobalt metal and a paste of lead linoleates containing 55 18% lead metal. The proportions are nine parts by weight of the former to six parts by weight of the latter. The amount of this mixture added to the oil is varied from 5% to 10% by weight depending on the particular grade of sandpaper 60 that is to be made. The coarse grades require a thicker film of oil, and, therefore, need more of the drying agent.

An illustrative example of carrying my invention into practice will be described hereinafter, 70 although it is to be understood that the scope of the invention is not to be limited by the materials and amounts given in this example.

I take a given quantity of the very viscous 75 polymerized oil made by the vacuum method and thin it with varnolene or petroleum spirits to

the desired viscosity. An appropriate amount of the paste driers, above mentioned, is weighed out and thinned with varnolene to the desired consistency. After proper thinning the driers are mixed and thoroughly incorporated in the 5 thinned polymerized oil. The paper or fabric to be coated with abrasive is well impregnated with this thinned solution of polymerized oil containing driers and is then dried on racks preferably by means of heated air. After the impregnated 10 fabric is dried it is re-rolled and passed through the coating machine again, printed on one side and coated on the opposite surface with the solution. Immediately thereafter it is sprinkled or 15 covered with a coating or layer of abrasive particles which are preferably of a predetermined size. The abrasive employed may be selected to meet the required conditions and may be an artificial abrasive such as silicon carbide, aluminum oxide, or the like, or a natural abrasive such as 20 garnet, flint, or the like. The abrasive paper is again carried along on racks into a heated chamber maintained at about 150° F. by heated air. After the oil film has acquired its set, which 25 usually takes approximately several hours, the paper is again passed through the machine for the application of a final sizing coat of polymerized oil to envelope the sand surface. When 30 this sizing coating is dried by air, heated to about 150° F., the abrasive fabric or sandpaper is taken 35 from the drying racks and is then cut into small sheets or small rolls which are ready for use or for sale in the markets.

In some instances where the coating surface of the primary fabric or paper is very porous, such 35 as very absorbent paper or cloth products, I add to the binder of oil and drier hereinbefore described, an inert filler material such as clay, fuller's earth, or other appropriate material. The filler imparts body to the binder and prevents 40 the latter from being easily absorbed.

It is to be noted that my invention provides an abrasive fabric containing a binder substance which consists practically wholly of a polymerized oil that has but little oxidation and further polymerization to undergo before setting to a tough, 45 extremely flexible, and durable film. Due to the polymerization of the oil, the film does not age in storage and the abrasive fabric retains its flexibility and toughness.

50 I claim:

1. A waterproof abrasive fabric having a flexible character comprising a waterproof fabric base, and a film in the nature of a matrix containing abrasive particles and consisting of polymerized oil, lead linoleate and cobalt linoleate, 55 united to said fabric base to form an integral product.

2. A waterproof abrasive fabric having a flexible character comprising a fabric base, and a film in the nature of a matrix containing a layer of abrasive particles and consisting of polymerized oil, lead linoleate, cobalt linoleate, lead 60 resinate, and cobalt resinate adhesively secured to a surface of said fabric base.

3. A waterproof abrasive fabric having a flexible character comprising a waterproof impregnated fabric base, and a film in the nature of a matrix containing a layer of abrasive particles and consisting of polymerized oil, driers, and 65 inert filler material incorporated on a surface of said fabric base.

4. A waterproof abrasive fabric having a flexible character comprising a waterproof impregnated fabric base, and a film in the nature of a 70 75

matrix containing abrasive particles and consisting of an extremely flexible, waterproof, polymerized and partly oxidized linseed oil containing a mixture of linoleates and resinates of lead and cobalt, said material being constituted to retain flexibility for a period of industrial storage.

5. An abrasive fabric comprising a base constituted of a fabric, a film coating containing an oil covering a surface of said fabric and a plurality of abrasive particles embodied in said film coating of such oil, said oil coating being characterized by having a minimum oxygen absorption factor during setting, resulting from pre-polymerization whereby flexibility of the fabric and coating will be retained throughout prolonged periods of storage of said abrasive fabric.

6. An abrasive fabric comprising a fabric base protected by a waterproof agent, a film coating superimposed upon a surface of said base containing an oil and abrasive particles anchored in said film coating, said film coating being characterized by including an oil having a minimum oxygen absorption factor during setting, resulting from prepolymerization whereby flexibility of the fabric and film coating will be retained throughout prolonged periods of storage of said abrasive fabric.

7. An abrasive fabric comprising a fabric base impregnated with an oil and a superimposed film coating of such oil, the superimposed coating including abrasive particles, said impregnated oil and film coating being characterized by having a minimum oxygen absorption factor during setting resulting from pre-polymerization, whereby said abrasive fabric will be extremely flexible and will retain said flexibility throughout prolonged periods of storage.

8. An abrasive fabric comprising a fabric base, a film coating containing an oil, a second film coating including a layer of abrasive particles secured thereto and a film coating containing an oil for the last layer superimposed over said abrasive particles, all of said film coatings being characterized by the oil thereof having a minimum oxygen absorption factor during setting, resulting from pre-polymerization whereby flexibility of the fabric and film coatings will be retained throughout prolonged periods of storage.

9. An abrasive fabric comprising a fabric base, a film coating of an oil including a drying agent covering the surface of said fabric, a layer of abrasive particles embedded in said film coating and a coating similar to said first coating superimposed over said abrasive particles, the oil of said film coating on said fabric and abrasive particles being characterized by having a minimum oxygen absorption factor during setting, resulting from prepolymerization whereby a flexible abrasive fabric is obtained, retaining the flexibility throughout prolonged periods of storage.

10. An abrasive fabric comprising a fabric base impregnated with an oil, a film coating consisting of an oil and a drying agent covering said impregnated fabric, abrasive particles anchored in said last film coating and presenting an abrasive surface and an enveloping film coating for said abrasive surface consisting of an oil and a drying agent, the oil of said impregnating layer, the film coating and the enveloping film coating being characterized by having a minimum oxygen absorption factor during setting, resulting from pre-polymerization whereby extreme flexibility of the entire abrasive fabric will be obtained and retained throughout prolonged periods of storage.

75 11. A waterproof abrasive fabric comprising a

waterproof impregnated fabric base, a layer of abrasive grains adhesively united to said base and a film coating consisting of an oil and a drying agent superimposed over said abrasive grains, said oil of said film coating being characterized by having a minimum oxygen absorption factor during setting resulting from pre-polymerization whereby flexibility of the product and coating will be retained throughout prolonged periods of storage of said abrasive fabric.

10 12. The process of making a waterproof abrasive fabric having a flexible character, which comprises preparing a viscous oil polymerized to a condition where the absorption of oxygen during subsequent setting of said oil is minimized and having a consistency amenable to retaining a layer of abrasive particles, thinning said oil to a consistency for spreading, applying the thinned polymerized oil in the form of a film to a dried fabric base impregnated with a waterproofing agent and incorporating a layer of abrasive particles in said film.

15 13. The process of making a waterproof abrasive fabric having a flexible character which comprises preparing a viscous oil by polymerization, the polymerization being carried to a condition where the absorption of oxygen during subsequent setting of said oil is minimized and having a consistency for retaining a layer of abrasive particles when in film form, thinning said oil to a consistency appropriate for spreading to a fabric base, applying a film of the aforementioned thinned, polymerized oil to a fabric base which has been previously impregnated with a waterproofing agent and dried, incorporating a layer of abrasive particles in said film, drying the fabric thus prepared to a condition leaving the oil film flexible and then applying over the composite film including the abrasives an additional coat of such polymerized oil first prepared and drying said coat, leaving the last coating of substantially the same flexibility as the first film.

20 14. The process of making waterproof abrasive fabrics having a flexible character which comprises preparing a viscous oil by polymerization to a condition where absorption during subsequent setting of the oil is minimized and having a body appropriate for retaining a layer of abrasive particles, thinning said oil to a consistency appropriate for application to a fabric by spreading, adding a drying agent to the polymerized oil so thinned and spreading a film of this mixture to an impregnated and waterproofed fabric base and incorporating a layer of abrasive particles to said film.

25 15. The process of making waterproof abrasive fabrics having a flexible character which comprises preparing a viscous oil by polymerizing to a condition whereby absorption of the oxygen during the subsequent setting of said oil is minimized, the polymerization being carried to an extent where it has body sufficient to carry a layer of abrasive particles, thinning said oil to a consistency appropriate for spreading to a fabric base, adding a drying agent to said polymerized oil so thinned, impregnating a fabric base with the aforesaid thinned polymerized oil, subjecting the fabric base so treated to the action of hot air to dry said fabric, leaving the fabric and oil mounted thereon flexible, applying a second coating of the aforesaid thin oil and coating a layer of abrasive particles thereover, and then drying the fabric including the coating of abrasive particles to a condition leaving the entire composite flexible.